



US006521172B2

(12) **United States Patent**  
Grearson et al.

(10) **Patent No.:** US 6,521,172 B2  
(45) **Date of Patent:** Feb. 18, 2003

(54) **TOOL FOR DRILLING/ROUTING OF PRINTED CIRCUIT BOARD MATERIALS**

(75) Inventors: **Alistair Grearson**, West Midlands (GB); **John Aucote**, Warks (GB)

(73) Assignee: **Sandvik AB**, Sandviken (SE)

(\*) Notice: Subject to any disclaimer, the term of this patent is extended or adjusted under 35 U.S.C. 154(b) by 53 days.

(21) Appl. No.: **09/486,586**

(22) PCT Filed: **Sep. 4, 1998**

(86) PCT No.: **PCT/SE98/01574**

§ 371 (c)(1),  
(2), (4) Date: **May 15, 2000**

(87) PCT Pub. No.: **WO99/13121**

PCT Pub. Date: **Mar. 18, 1999**

(65) **Prior Publication Data**

US 2002/0031440 A1 Mar. 14, 2002

(30) **Foreign Application Priority Data**

Sep. 5, 1997 (SE) ..... 9703204

(51) **Int. Cl.<sup>7</sup>** ..... C22C 32/00

(52) **U.S. Cl.** ..... 419/18

(58) **Field of Search** ..... 419/18

(56) **References Cited**

**U.S. PATENT DOCUMENTS**

3,994,716 A 11/1976 Huppmann et al. ..... 75/5 BB  
4,093,450 A 6/1978 Doyle et al. ..... 75/5 AA  
4,469,505 A 9/1984 Cheresnowsky et al. ... 75/5 BA  
4,539,041 A \* 9/1985 Figlarz et al.

4,574,011 A \* 3/1986 Bonjour et al.  
5,476,531 A \* 12/1995 Timm et al. ..... 75/240  
5,482,530 A 1/1996 Hohne ..... 75/230  
5,603,075 A \* 2/1997 Stoll et al.  
5,658,678 A 8/1997 Stoll et al.  
5,802,955 A 9/1998 Stoll et al.  
6,015,447 A 1/2000 Gorge et al. ..... 75/255

**FOREIGN PATENT DOCUMENTS**

|    |           |           |
|----|-----------|-----------|
| AT | 268706    | * 2/1969  |
| DE | 2225896   | * 12/1972 |
| DE | 27 19 532 | 11/1977   |
| GB | 622041    | * 4/1949  |
| GB | 1309634   | * 3/1973  |
| WO | 9213112   | * 8/1992  |
| WO | 9218656   | * 10/1992 |

**OTHER PUBLICATIONS**

V.A. Tracey et al., "Development of Tungsten Carbide-Co-balt-Ruthenium Cutting Tools for Machining Steels," vol. 82, No. 1, 1998, XP000574252, pp. 281-292.

B. Zetterlaund, "Cemented Carbide in High Pressure Equipment," *High Pressure Engineering*, vol. 2, 1977, pp. 35-40.

\* cited by examiner

*Primary Examiner*—Daniel J. Jenkins

(74) *Attorney, Agent, or Firm*—Burns, Doane, Swecker & Mathis, L.L.P.

(57) **ABSTRACT**

A dense cemented carbide product is described. The product is manufactured from WC with a grain size between 0.1 and 0.4 ¼ m, fine grain size cobalt and ruthenium powders. The product is used in PCB machining operations where the addition of 10-25% Ru to the binder phase offers up to 25% wear resistant increases and up to 100% increase in chipping resistance in PCB routing compared to conventional materials (6% cobalt and 0.4 ¼ m grain size).

**11 Claims, No Drawings**

## TOOL FOR DRILLING/ROUTING OF PRINTED CIRCUIT BOARD MATERIALS

The present invention relates to a tool for drilling/routing of printed circuit board materials. By alloying the binder phase with Ru in combination with the use of fine grained Co-powder the properties have been improved.

Cemented carbide containing Ru as binder phase alone or in combination with the conventional Co and/or Ni is known in the art. For example, AT 268706 discloses a hard metal with Ru, Rh, Pd, Os, Ir, Pt and Re alone or in combination as binder phase. U.S. Pat. No. 4,574,011 discloses a hard metal composition for ornamental purposes with a binder phase of Co, Ni and Ru. GB 1309634 discloses a cutting tool with a Ru binder phase. GB 622041 discloses a hard metal composition a Co+Ru binder phase.

The routing of Printed Circuit Board materials requires a wide range of properties from the tool material in order for it to perform successfully. These include a hardness in excess of 2000 HV, a resistance to edge chipping that is best defined by a fracture toughness in excess of 8 MPam<sup>1/2</sup>, a resistance to chemical attack from the resins included in printed circuit boards and a sharp as possible a cutting edge. Some of these requirements conflict, for instance the high hardness tends to mean a reduced edge toughness. The new products for this application can, therefore, require a reduced WC grain size to produce a higher hardness with reduced toughness. However, if this is combined with an increase in cobalt content an increased toughness can be achieved for the same hardness. This also results in a sharper cutting edge, which is required.

The invention is primarily concerned with the addition of ruthenium to submicron grades of cemented carbide. The levels of addition vary between 5 and 35, preferably between 15 and 30, wt-% of the binder content with the best results obtained at about 25 wt-%. For best effects the cobalt used should be of the fine grain size cobalt powder having deagglomerated spherical grains of about 0.4  $\mu\text{m}$  average grain size and with a narrow grain size distribution. Preferably the cobalt powder is polyol cobalt. The cobalt contents to which this addition can be made should vary from 5–12%, preferably 5–8. The average WC grain size shall be <0.8  $\mu\text{m}$ , preferably <0.4  $\mu\text{m}$ . The cemented carbide of the invention is preferably a straight WC+Co grade but it may also contain <5 wt-% gammaphase.

In order to obtain the submicron WC grain size 45 VC+Cr<sub>3</sub>C<sub>2</sub> is added. Because the Ru also acts as a mild grain growth inhibitor an addition of <0.9 wt % VC+Cr<sub>3</sub>C<sub>2</sub> is generally satisfactory. Particularly good results are obtained if the VC/Cr<sub>3</sub>C<sub>2</sub> ratio in wt % is 0.2–0.9, preferably 0.4–0.8, most preferably 0.6–0.7. Preferably sintering is performed 50 using gas pressure sintering also referred to as sinter-HIP.

The invention also relates to the use of a cemented carbide with submicron WC grain size and with a binder phase containing 10–30 wt-% Ru as a tool for drilling/ routing of printing circuit board materials.

The present invention further relates to a method of making a cemented carbide body comprising one or more hard constituents and a binder phase based on cobalt, nickel and/or iron by powder metallurgical methods milling, pressing and sintering of powders forming hard constituents and binder phase whereby said binder phase contains 10–30 wt-% Ru. At least part of the binderphase powder consists of non agglomerated particles of spheroidal morphology of about 0.4  $\mu\text{m}$  average grain size and with a narrow grain size distribution wherein at least 80% of the particles have sizes 55 in the interval  $x \pm 0.2 x$  provided that the interval of variation (that is 0.4 x) is not smaller than 0.1  $\mu\text{m}$ .

The advantages offered by the ruthenium additions are as mentioned a further element of grain growth refinement, an increase in resistance to chemical attack and a strengthening of the binder phase without significantly affecting the edge toughness due to the increase in cobalt content used.

### EXAMPLE 1

Cemented carbide PCB-router according to the invention were made with the composition 1.9% Ru, 5.6% Cobalt the 10 remainder WC (0.2  $\mu\text{m}$  grain size), with about 0.7% (VC+Cr<sub>3</sub>C<sub>2</sub>) grain growth inhibitor. The material had a hardness of 2080 HV and a KIC of 8.75 MPam<sup>1/2</sup>.

For comparison the following PCB routers according to prior art were also made. One was 6% cobalt grade with 0.4 15  $\mu\text{m}$  WC with a hardness of 2000–2100 HV and one with the same hardness but with 5% cobalt and 0.5  $\mu\text{m}$  WC grain size.

The routers were ground to 2.4 mm dia and tested as follows:

20 Workmaterial: Copper clad 3 mm thick FR4 PCB, stacked three deep

Test 1: 30,000 RPM, 1.2 m/min feedrate, 150 m of cut

Test 2: 42,000 RPM, 2.2 m/min feedrate, 100 m of cut

25 In test 1 routers according to the invention reached 150 m of cut with 25% less average wear than the prior art routers which used 6% cobalt.

In test 2 routers according to the invention reached 100 metres of cut with acceptable levels of wear.

30 Routers according to prior art with 5% and 6% cobalt both fractured between 50 and 75 metres.

### EXAMPLE 2

2.4 mm dia routers according to the invention were made 35 from cemented carbides with varying ruthenium contents as follows:

Composition 1: 1.0% Ru, 6.3% Co, 0.7 VC+Cr<sub>3</sub>C<sub>2</sub>, 0.2  $\mu\text{m}$  WC

Composition 2: 1.4% Ru, 6.0% Co, 0.7 VC+Cr<sub>3</sub>C<sub>2</sub>, 0.2  $\mu\text{m}$  WC

Composition 3: 1.9% Ru, 5.6% Co, 0.7 VC+Cr<sub>3</sub>C<sub>2</sub>, 0.2  $\mu\text{m}$  WC

The routers were tested as follows:

Workmaterial: Copper clad 3 mm thick FR4 PCB, stacked three deep

Conditions : 30,000 RPM, 1.2 m/min feed rate.

Machining until fracture.

Results:

1.0% Ru variant—205 m (Average of 4 cutters)

1.4% Ru variant—333 m (Average of 5 cutters)

1.9% Ru variant—366 m (Average of 7 cutters)

### EXAMPLE 3

55 Cemented carbide PCB microdrills according to the invention were made with the composition 2.2% Ru, 6.4% Co the remainder WC (0.4  $\mu\text{m}$  grain size), with about 0.8% (VC+Cr<sub>3</sub>C<sub>2</sub>) grain growth inhibitor. The material had a hardness of 2010 HV and a KIC of 8 MPam<sup>1/2</sup>.

60 For comparison the following PCB micro drills according to prior art were made using 8% cobalt grade with 0.4  $\mu\text{m}$  WC with a hardness of 1900 HV.

The microdrills were tested and the wear measured. It was found that the prior art materials exhibited 10–15% less wear resistance and 10–15% less resistance to breakage during an increasing feed rate that started at 15  $\mu\text{m}/\text{rev}$  and increasing towards 70.

What is claimed is:

1. Method of making a cemented carbide body comprising one or more hard constituents and a binder phase by pressing and sintering of powders forming hard constituents and binder phase whereby said binder phase contains 10–30 wt. % Ru wherein at least part of the binder phase powder comprises non agglomerated particles of spheroidal morphology of about  $0.4 \mu\text{m}$  average grain size and with a narrow grain size distribution wherein at least 80% of the particles have sizes in the interval  $x \pm 0.2x$  provided that the interval of variation of  $0.4x$  is not smaller than  $0.1 \mu\text{m}$ .

2. Cemented carbide comprising 5–12% Co binder phase formed from Co powder having deagglomerated spherical grains with a grain size distribution such that at least 80% of the grains have sizes in the interval  $x \pm 0.2x$ , provided that the interval of variation of  $0.4x$  is not smaller than  $0.1 \mu\text{m}$ , wherein said binder phase contains 10–30 wt. % Ru, and submicron WC.

3. Cemented carbide according to claim 2, wherein the deagglomerated spherical grains have an average grain size of about  $0.4 \mu\text{m}$ .

4. Cemented carbide according to claim 2, further comprising VC in an amount greater than zero,  $\text{Cr}_3\text{C}_2$  in an amount greater than zero, such that  $(\text{VC}+\text{Cr}_3\text{C}_2)$  is in an amount greater than zero and less than 0.9 wt. %.

5. Cemented carbide according to claim 4, wherein the ratio of wt. % defined as  $\text{VC}/\text{Cr}_3\text{C}_2$  is 0.2–0.9.

6. Method according to claim 1, wherein the powders further comprise VC in an amount greater than zero,  $\text{Cr}_3\text{C}_2$  in an amount greater than zero, such that  $(\text{VC}+\text{Cr}_3\text{C}_2)$  is in an amount greater than zero and less than 0.9 wt. %.

7. Method according to claim 6, wherein wherein the ratio of wt. % defined as  $\text{VC}/\text{Cr}_3\text{C}_2$  is 0.2–0.9.

8. A machining tool comprising cemented carbide with 5–12% Co binder phase formed from Co powder having deagglomerated spherical grains with a grain size distribution such that at least 80% of the grains have sizes in the interval  $x \pm 0.2x$ , provided that the interval of variation of  $0.4x$  is not smaller than  $0.1 \mu\text{m}$ , wherein said binder phase contains 10–30 wt. % Ru, and submicron WC.

9. Machining tool according to claim 8, wherein the deagglomerated spherical grains have an average grain size of about  $0.4 \mu\text{m}$ .

10. Machining tool according to claim 8, further comprising VC in an amount greater than zero,  $\text{Cr}_3\text{C}_2$  in an amount greater than zero, such that  $(\text{VC}+\text{Cr}_3\text{C}_2)$  is in an amount greater than zero and less than 0.9 wt. %.

11. Machining tool according to claim 10, wherein the ratio of wt. % defined as  $\text{VC}/\text{Cr}_3\text{C}_2$  is 0.2–0.9.

\* \* \* \* \*